

## UNITED STATES PATENT OFFICE.

LEWIS DAVIS, OF WORCESTER, AND ELMER W. BENNETT, OF WESTBORO, MASSACHUSETTS, ASSIGNORS TO DAVIS & BENNETT, INC., OF WORCESTER, MASSACHUSETTS, A CORPORATION OF MASSACHUSETTS.

## WAX EMULSION.

No Drawing.

Application filed December 2, 1924. Serial No. 753,430.

This invention consists of a wax emulsion, and of a process of producing the same. Its object is more particularly to provide an emulsion which will serve as a lubricant for 5 thread, such as used in sewing together certain portions of footwear, which will perform the desired function without discoloring the thread, where such discoloration is undesirable. The emulsion for this purpose 10 should be of such consistency and viscosity that in drawing the thread therethrough, it will be supplied with only the necessary amount of the lubricant, without the formation of an excess at the apertures in the 15 leather or other material through which the thread is passed.

Any suitable wax or waxlike body may be emulsified for this purpose such as japan, spermaceti, shellac or ceresin waxes or 20 beeswax, but preferably we use carnauba wax, which to hasten the process, is mechanically comminuted before subjecting it to the emulsifying or dispersing process.

We employ, as the stabilizing, emulsifying, or dispersing agent, a colloidal material 25 which is a mixture of hard and soft soaps, preferably stearates. We have found that results are secured by this agent which are superior to those resulting from the use of 30 either a hard soap or a soft soap. Preferably, as stated, this soap consists of a mixture of sodium stearate and potassium stearate, and it is produced by the reaction of stearic acid with sodium and potassium alkalis. 35 For example, about 18.75 parts (by weight) of potassium carbonate ( $K_2CO_3 \cdot 2H_2O$ ) and about 6.75 parts of sodium carbonate ( $Na_2CO_3 \cdot H_2O$ ) is dissolved in about 1000 parts of water. To this solution we add 40 about 50 parts by weight of stearic acid (preferably triple pressed) in relatively small pieces. The mass is heated slowly with constant agitation until the solution is effected, precautions being observed to prevent too violent reaction between the carbonates and the acid. The heating is continued until the solution begins to boil. We now add to the boiling solution the wax which is to be dispersed or emulsified. If 45 the product is to be employed as a lubricant for thread, we preferably use carnauba wax, in which case it is usually ground or comminuted to about 20 mesh size, and about 50 11.25 parts are added to the solution, while

at the same time the heating and strong agitation of the mass are continued until the wax has been dispersed. The vessel in which the dispersion is effected, is preferably jacketed for the circulation of the steam, and when the dispersion has been effected, a 55 cooling or refrigerating medium is circulated through the jacket for the purpose of rapidly chilling the mass, while at the same time the agitation is continued. When the mass has reached a temperature of about 65° C. it is now strained through cheese cloth to remove any large particles, and then allowed to cool slowly to room temperature. On standing for about 20 hours, the product 60 is a white milky liquid of colloidal consistency—of about the viscosity of “cylinder oil” so called. When produced in accordance with the foregoing example, the product, at 70° F. has a viscosity of 1.34 (Engler) and at 212° F. of 1.09. It is slightly alkaline, having a reaction of PH around 10. It is miscible with and may be diluted with 65 water to any reasonable or required extent. When heated above 65° C., the liquid becomes 70 nearly transparent, of much thinner consistency and turns from white to straw yellow but on being cooled returns to its original condition. When subjected to a temperature below —4° C., it begins to precipitate as a result of freezing.

In the operation hereinbefore described, the wax which softens and melts at the temperature of the soap solution into which it is introduced, is already in relatively small particles, but with the strong agitation it is 75 finally dispersed in particles of substantially colloidal size, and on being rapidly chilled while the agitation is continued, the resultant product after reaching a temperature of about 65° C. is remarkably stable. It is of 80 such consistency that when a thread is drawn therethrough, it picks up just sufficient lubricant to permit the manipulation of the thread in the sewing operation, to the best 85 advantage.

After prolonged experimentation with the use of soaps, in producing dispersions, we discovered that by using a blend of hard and soft soaps, a final product could be obtained having the proper fluidity or consistency, and having such a slight total alkalinity as would not affect the thread. While we do not desire to be understood as limit- 90 95 100 105

ing ourselves to the use of a specific fatty acid, or to exact proportions of the blended soaps, or to the exact ratio of soap to wax and water, yet we regard the proportions herein stated to be the best for our specific purpose. An amount of wax in excess of that stated, does not produce a stable unchanging dispersion, while a smaller amount does not give the best lubricating value to the product.

For other specific uses, we may employ other thermoplastic waxes or gums or bodies normally immiscible with water which may be initially softened by or dissolved in suitable solvents if desired, before their being added to the water containing the blended-soap colloid. Where discoloration of the thread to be lubricated by the dispersion is

undesirable, one should employ a light colored wax, rather than a material such as asphalt.

What we claim is:

1. A dispersion consisting of carnauba wax dispersed in water, and a mixture of sodium and potassium stearates serving as the dispersing agent.

2. A lubricant for thread, comprising a carnauba wax dispersion in water containing a mixture of sodium and potassium stearates as the dispersing agents, and having a viscosity of about 1.34 (Engler) at 70° F.

In testimony whereof we have affixed our signatures.

LEWIS DAVIS.  
ELMER W. BENNETT.